

## UNITED STATES PATENT OFFICE

FERNANDO SOMOZA VIVAS, OF NEW YORK, N. Y., ASSIGNOR TO INTERNATIONAL FIRE-PROOF PRODUCTS CORPORATION, OF NEW YORK, N. Y., A CORPORATION OF DELAWARE

## FIREPROOF WALL BOARD AND PROCESS OF PRODUCING THE SAME

No Drawing.

Application filed October 8, 1927. Serial No. 225,038.

The invention relates to wallboard which shall be fireproof and substantially waterproof and which may be produced from any suitable cellulose material such as bagasse, 5 wood pulp, cornstalks, straw or the like.

It is an object of the invention to provide wallboard having the qualities named and which will be cheap to produce.

It is a further object of the invention to 10 provide wallboard of this character which shall have excellent sound and heat insulating qualities and at the same time shall be fireproof or exceedingly fire-resistant.

It is a further object of the invention to 15 provide material of the character described which will be a suitable substitute for lumber in the construction of buildings.

Further objects of the invention will appear from the following description disclosing 20 an illustrative embodiment of the invention.

The process of the invention may be carried out by preparing a pulp of any suitable cellulose material such as bagasse, wood pulp or 25 the like. In a desirable embodiment of the invention there is added to each pound of the dried pulp one-half pound of calcium chloride dissolved in sufficient water to provide a perfect saturation of pulp without the 30 water running from the pulp when it is handled.

After such a saturated pulp has been produced, there is added to the pulp a solution comprising resinated soap to the amount of 35 one ounce to each pound of dried pulp producing in the pulp a calcium resinate soap binder.

After thorough mixing of the soap solution with the pulp, the material is flowed with a 40 strong solution of aluminum sulphate. A solution of suitable strength may be provided by dissolving two pounds of sulphate in a gallon of water. If desired, ammonia alum may be substituted for the aluminum sulphate. The last named solution acting upon 45 the soap binder already named will cause the same to be insoluble in water, and leave the pulp in condition to be pressed or rolled into shape as wallboard.

The thus treated pulp is formed into a

sheet in any usual manner, the sheet when formed being desirably about one inch in thickness after which it is pressed or rolled into the shape of wallboard to reduce its thickness to substantially three-fourths of an 55 inch.

The compressed sheets are then dried to evaporate the water when the sheets will shrink to a thickness of practically one-half inch and the spaces in the sheet formerly occupied by the water will leave the sheet in a porous condition.

The thus produced board is exceedingly fire-resistant, waterproof, cheap and easy to manufacture and is highly sound insulating and heat insulating. Plaster may be applied directly to such wallboard when in place in 60 buildings.

In addition to its porosity and cheapness, the wallboard is flexible and of light weight 70 and forms an exceedingly desirable material for use in the building arts.

Minor changes may be made in the composition of the material or in the steps of the process of preparing the same, within the scope of the appended claims without departing from the spirit of the invention.

I claim:

1. A wallboard comprising a porous body of cellulose material impregnated with an 80 insoluble calcium resinate soap binder.

2. A wallboard comprising a porous compressed body of cellulose material impregnated with a calcium resinate soap binder 85 rendered insoluble by treatment with an aluminum sulphate.

3. The process of producing wallboard which comprises saturating a pulp of cellulose material with a solution of calcium chloride, adding resinated soap to the thus treated pulp, treating the thus prepared material with a substance adapted to make the calcium soap binder insoluble and compressing the material into sheets.

4. The process of producing wallboard which comprises treating cellulose pulp with a solution of calcium chloride, treating the thus treated pulp with resinated soap, flowing the thus treated material with a solution of 100

an aluminum sulphate and forming the material into sheets.

5. The process of producing wallboard which comprises saturating cellulose pulp with a calcium chloride solution, adding a solution of a resinated soap to the thus prepared pulp, flowing the thus treated material with a strong solution of aluminum sulphate, compressing the material into sheets and drying the sheets.

**FERNANDO SOMOZA VIVAS.**

**15****20****25****30****35****40****45****50****55****60****65**